

## UNITED STATES PATENT OFFICE

FREDERICK G. MOSES, OF NEW YORK, RAYMOND W. HESS, OF BUFFALO, AND ROBERT L. PERKINS, OF EAST AURORA, NEW YORK, ASSIGNORS TO THE BARRETT COMPANY, OF NEW YORK, N. Y., A CORPORATION OF NEW JERSEY

## SEPARATION OF MINERALS

No Drawing.

Application filed May 20, 1927. Serial No. 193,059.

This invention relates to the separation of minerals and the concentration of ores by flotation processes, and is particularly directed to such separation and concentration carried out with the utilization of certain thiobiazoline compounds, or derivatives thereof, as flotation or mineral collecting agents.

According to the present invention, improved results can be obtained in the separation of minerals and the concentration of ores by carrying out the flotation operation with the addition to the ore or mineral pulp of a thiobiazoline sulfhydrate body or compound which embodies within its composition the following probable atomic grouping:



Bodies or compounds containing this grouping may also be designated as derivatives of 5-mercaptop-2,3-dihydro-1,3,4-thiodiazol which corresponds with the following probable formula:



Of particular importance for use as flotation agents according to the present invention are those thiobiazolines having the following probable general formula:



wherein R denotes a monovalent hydrocarbon radical, particularly an aryl group and especially an aryl group of the benzene series. 5-mercaptop-3-phenyl-2-hydro-1,3,4-thiodiazole, i. e., phenylthiobiazoline sulfhydrate, is particularly important. The thiobiazoline sulfhydrates may be prepared by methods described in chemical literature.

In carrying out the flotation process, the flotation agent comprising the thiobiazoline sulfhydrate compound may be incorporated with the ore or mineral pulp in any suitable

manner and at any suitable time which will insure a satisfactory flotation operation. For example, it may be introduced in the free state or as a salt into the mill in which the ore is being ground, or it may be dissolved, suspended or dispersed in any suitable solvent or dispersing agent as, for example, in one or more of the usual flotation oils or oil mixtures, or in any suitable organic solvent or medium, or in water or in an alkali or alkaline reagent, and the resulting solution, dispersion, or dispersion incorporated with the ore or mineral pulp. While the agents of the present invention show marked action as flotation or collecting agents in ore concentration, they ordinarily possess insufficient frothing qualities and are therefore generally used to advantage in conjunction with any suitable or well known frothing agent, e. g., pine oil, crude turpentine, coal tar acid, etc. They may be also sometimes used to advantage in connection with other flotation agents. They may be used in the pure or purified state; and, in general, they may be also employed in the crude or impure state.

The process of the present invention may be carried out in any suitable apparatus as, for example, those of the pneumatic type such as the Callow cell, or those in which the air is incorporated with the mixture by agitation such as the Janney apparatus, or the like.

It is of advantage in some cases, as with certain copper ores, to subject the ore pulp to the action of an amount of alkali sufficient to give it an alkaline reaction before subjecting it to flotation with the aid of the flotation agents of the present invention. The alkali may be caustic alkali such as caustic soda, or an alkaline salt such as soda ash, or it may be calcium oxide or hydrate.

In the differential separation of various minerals, such as zinc blende from associated minerals, the presence of an alkali metal cyanide, or of copper sulfate or other salts, is sometimes advantageous.

The amount of flotation agent required to be used in the flotation process will vary, it depending partly on the character and composition of the ore, partly on the particular thiobiazoline sulfhydrate compound employed, and partly on other factors. Ordinarily, one-sixth to one-half pound of the flotation agent per ton of dry ore will be sufficient, but larger or smaller amounts than this may be used.

The invention will be further illustrated by the following specific example, but it will be understood that the invention is not limited thereto. The parts are by weight.

Example: 500 parts of a copper sulfide ore (of the Miami Copper Co.) assaying 1.18 percent copper, was ground in a ball mill with 300 parts of water and 0.75 parts of hydrated lime (equivalent to 3 pounds per ton of ore) until practically all of it was sufficiently fine to pass through a 40-mesh screen. The ground pulp was diluted with sufficient water to give a pulp containing about 16 percent solids and subjected to flotation in a Janney mechanical apparatus with the addition of 0.0625 parts of phenylthiobiazoline sulfhydrate (equivalent to one-fourth pound per ton of ore) previously dissolved in an equivalent amount of normal caustic soda solution. The mixture was agitated for 30 minutes during which time about 0.06 parts of pine oil was introduced. 26.1 parts of a concentrate assaying 16.1 percent copper was obtained which is a recovery in the concentrate of 75.75 percent of the copper. The tailings assayed 0.28 percent copper. It will be noted that the equivalent of about 19.1 tons of ore was required to give one ton of concentrate.

It will thus be noted that the present invention contemplates the utilization as flotation agents in the separation of minerals and the concentration of ores of thiobiazoline sulfhydrate compounds; that said flotation agents may be incorporated in or with the ore or mineral pulp at any suitable time or in any suitable manner; that they may be used in the free state or as salts or in admixture with one another or in solution, suspension or dispersion in any suitable solvent or medium; and that they may be used in conjunction with other flotation agents or with frothing agents, or with both.

The present invention is of more or less general application to the treatment of different kinds of mineral substances, both natural and artificial, by flotation.

It will be further understood that the invention is not limited to the use of the particular agents or ingredients mentioned in the example and that other agents, particularly other flotation agents of the class specified, can be used.

We claim:

1. In effecting the separation of miner-

als, the process which comprises incorporating with the mineral pulp a thiobiazoline sulfhydrate compound which embodies within its composition the following probable grouping:



and subjecting the resulting mixture to a froth flotation operation.

2. In effecting the separation of minerals, the process which comprises incorporating with the mineral pulp a thiobiazoline compound corresponding with the following probable formula:



where R denotes a monovalent hydrocarbon radical, and subjecting the resulting mixture to a froth flotation operation.

3. In effecting the separation of minerals, the process which comprises incorporating with the mineral pulp a thiobiazoline compound corresponding with the probable formula:



where R denotes an aryl group, and subjecting the resulting mixture to a froth flotation operation.

4. In effecting the separation of minerals, the process which comprises incorporating with the mineral pulp a thiobiazoline compound corresponding with the probable formula:



where R denotes an aryl radical of the benzene series, and subjecting the resulting mixture to a froth flotation operation.

5. In effecting the separation of minerals, the process which comprises incorporating phenylthiobiazoline sulfhydrate with the mineral pulp, and subjecting the resulting mixture to a froth flotation operation.

6. In effecting the separation of minerals, the process which comprises incorporating with a copper sulfide ore pulp a thiobiazoline sulfhydrate compound which embodies within its composition the following probable grouping:



and subjecting the resulting mixture to a froth flotation operation.

7. In effecting the separation of minerals, the process which comprises incorporating with a copper sulfide ore pulp a thiobiazoline compound corresponding with the following probable formula:



where R denotes a monovalent hydrocarbon

radical, and subjecting the resulting mixture to a froth flotation operation.

8. In effecting the separation of minerals, the process which comprises incorporating 5 phenylthiobiazoline sulfhydrate with a copper sulfide ore pulp and subjecting the resulting mixture to a froth flotation operation.

In testimony whereof we affix our signatures.

10                   FREDERICK G. MOSES.  
                      RAYMOND W. HESS.  
                      ROBERT L. PERKINS.

15

20

25

30

35

40

45

50

55

60

65